



US005123350A

## United States Patent [19]

Fadner

[11] Patent Number: 5,123,350

[45] Date of Patent: Jun. 23, 1992

## [54] HYDROPHOBIC AND OLEOPHILIC MICROPOROUS INKING ROLLERS

[75] Inventor: Thomas A. Fadner, La Grange, Ill.

[73] Assignee: Rockwell International Corporation, El Segundo, Calif.

[21] Appl. No.: 689,086

[22] Filed: Apr. 19, 1991

## Related U.S. Application Data

[63] Continuation of Ser. No. 343,557, Apr. 27, 1989, abandoned.

[51] Int. Cl.<sup>5</sup> ..... B41F 31/26

[52] U.S. Cl. ..... 101/348; 29/121.8; 29/132; 29/895

[58] Field of Search ..... 101/348, 349, 350, 147, 101/148, 450.1, 451, 452; 427/333, 344, 230; 29/121.1, 121.8, 132, 895, 895.3, 895.32, 895.33

## [56] References Cited

## U.S. PATENT DOCUMENTS

4,301,730 11/1981 Heurich et al. .... 101/348  
4,601,242 7/1986 Fadner ..... 101/348

Primary Examiner—Clifford D. Crowder

Attorney, Agent, or Firm—C. B. Patti; V. L. Sewell; H. F. Hamann

## [57] ABSTRACT

An inking roller or ink metering roller comprised of a base roller, a substantially continuous hard and wear-resistant microporous ceramic coated layer bonded to the base roller and an interdiffused and immobilized oleophilic and hydrophobic essentially organic polymeric based material affixed to the surfaces and interstices of the microporous layer.

10 Claims, 2 Drawing Sheets



Fig. I.



Fig. 2.



Fig. 3.



Fig. 4.



Fig. 5.



Fig. 6.



## HYDROPHOBIC AND OLEOPHILIC MICROPOROUS INKING ROLLERS

This is a continuation of application Ser. No. 343,557, 5 filed Apr. 27, 1989, now abandoned.

### BACKGROUND OF THE INVENTION

In the practice of keyless inking for lithographic printing whereby ink is metered into the printed system 10 by means of a metering roller and a cooperating scraping blade, Fadner in U.S. Pat. No. 4,601,242, Fadner and Hycner in U.S. Pat. No. 4,537,127 and Fadner in U.S. Pat. No. 4,603,634 have disclosed advantageous 15 method and means wherein the surface of an ink metering roller will possess the dual property of being both hydrophobic and oleophilic, that is water-repelling and oil attracting. This dual property can be present whether the lithographic ink metering roller surface is formed with ink retaining dimensioned cells or is 20 formed with a surface possessing irregularly spaced cavities capable of retaining ink. In practicing keyless inking the presence of oleophilic and hydrophobic properties at the surface of the ink metering roller is vital, since lithography requires the presence of water in 25 the films of ink being used. The presence of hydrophilic, or water attracting regions on the ink metering roller surface will allow water to displace or debond ink from those regions, thereby disrupting the roller's ink carrying and ink metering capabilities.

The above-named Fadner, et al. prior art references also teach that even when consistent ink metering is assured by providing a metering roller surface that is both hydrophobic and oleophilic, the water contents of the ink films on the inking rollers may vary across the 30 press width, depending upon the relative amounts of ink and water consumed in satisfying the format being printed. To accomplish uniform ink availability across the press during a printing run, it is necessary to assure that a constant ink composition is continuously available to all portions of the printing plate. Unless constant ink composition is available across the press width, the water content tends to increase in regions of low print 35 density and undesirable print quality occurs. Means for obtaining press wide uniformity of ink composition are disclosed in the Fadner, et al U.S. Pat. No. 4,690,055.

When hydrophilic regions are purposefully included in either a random or in geometrically uniform manner, such as the land areas of the celled metering roller disclosed in U.S. Pat. No. 4,637,310 by Sato and Harada or 40 as in the non-celled or smooth-surfaced metering roller disclosed in U.S. Pat. No. 4,287,827 by Warner, it might be reasoned that predictability of ink metering will be achieved because any water interference due to debonding of ink from the hydrophilic regions would be in 45 accord with the pattern selected when forming the hydrophilic regions. However, the through-puts of water and ink across the press width and therefore the relative amounts of each required, are determined by the image and non-image format on the printing plate 50 being used at any given time. Printing formats are not uniform generally and are rarely the same from press-run to press run. Consequently, the extent of ink debonding by water when operating an apparatus utilizing the oleophilic and hydrophilic technology will depend 55 upon the instantaneous amounts of water present in the ink at various locations on the metering roller. These locations correspond in turn to the various cross press 60

ink and water amounts required to print the format on the printing plate. The higher the water content in the ink at a hydrophilic/region, the greater will be the propensity for loss of ink carrying capability because of debonding of ink in the corresponding localized region. The result is variable ink input from press-run to press-run as the printed format is changed, with concomitant printed regions of unexpectedly low or unexpectedly high optical density.

Hard ceramic materials, such as chromium and aluminum oxides and tungsten carbide are naturally high energy materials and correspondingly tend to be hydrophilic in the presence of water and tend to be oleophilic in the presence only of oily materials. Metering rollers manufactured using these materials, while often used successfully in conjunction with either water based inks or with oil based inks in letterpress printing, fail to deliver consistent quantities of ink during lithographic printing utilizing oil based inks having water present. The extent of ink delivery inconsistency is determined by whether water present in the ink has displaced or debonded ink from the roller's ceramic surface. As previously noted, the extent of debonding depends upon the water content of the ink at any selected cross-press location, which water content in turn depends upon the format being printed.

The previously referred to Fadner U.S. Pat. No. 4,601,242 discloses one means to use the advantageously hard and wear-resistant ceramic property to obtain 30 reasonably long lithographic ink metering roller lifetimes. Specifically, ceramic powder, and in particular alumina, is flame sprayed in a purposefully thin layer of less than about 2 mils thickness over a copper plated metering roller base. Copper is naturally hydrophobic and oleophilic. This procedure results in a hard, wear-resistant surface that has sufficient inter-particle porosity relative to ink and water interactions that the surface acts as if it was copper, therefore retaining ink in preference to water, yet simultaneously acts as a wear-resistant 35 ceramic material relative to scraping blade wearing action. Although commercially viable, this type of roll has a lifetime on a printing press of about 20 to 30 million printing impressions, because the ceramic layer must be kept relatively thin to assure that the oleophilic property of the underlying copper is not negated by the hydrophilic properties exhibited by the ceramic layer. Further, the ceramic layer, which is naturally hydrophilic, may become increasing hydrophilic due to accumulation of contaminants associated with use and cleaning 40 of printing presses.

A primary object of this invention is to provide a simple, inexpensive ink metering roller that ensures long operational lifetimes in keyless lithographic printing press systems where the presence of water in the ink is involved.

An additional object of this invention is to provide a process for producing an ink metering roll having a microporous wear-resistant surface layer that is infused with a substantially organic material that reacts to form a reaction product that is oleophilic and hydrophobic.

Still another object of this invention is to provide means whereby hard and wear-resistant but naturally hydrophilic ceramic materials can be used as part of a composite layer that has hydrophobic and oleophilic properties without detracting from their naturally excellent wear-resistant quality.

A further object of this invention is to provide an improved inking roller having a composite structure

that combines high degrees of wear resistance with a preferential attraction for and retention of oil inks in the presence of water.

Other objects and advantages of this invention will be in part obvious and in part explained by reference to the accompanying specification and drawing in which:

#### DESCRIPTION OF THE DRAWINGS

FIG. 1 is a schematic side elevation of keyless lithography printing system configuration illustrating a lithographic printing arrangement incorporating an ink metering roll of the present invention;

FIG. 2 is a sectional view through a portion of the roll of this invention showing the infused, wear resistant surface in which recesses to hold ink are provided;

FIG. 3 is a sectional view similar to FIG. 2 but with a roller having no individually formed ink receiving recesses;

FIG. 4 is a sectional view similar to FIG. 3 showing a variation in the shape of individually formed ink receiving recesses;

FIG. 5 is a plan view of FIG. 4; and

FIG. 6 is an enlarged illustration of a section through the microporous ceramic layer to show the location of the oleophilic and hydrophobic reaction product.

#### SUMMARY OF THE INVENTION

This invention relates to an improved ink metering roll for metering ink in modern, high-speed lithographic printing press systems, and to an inking system wherein keyless means are provided to simplify the inking system and to simplify the degree of operator control or attention required during operation of the printing press.

Typically, a press using a keyless inking system will comprise an ink reservoir or sump 10, a pump 11 and piping 12 interconnecting an ink pan 13, within which a metering roller 14 is located, to supply ink to a frictionally driven ink transfer roller 15. A reverse angle scraping or metering blade 16 operates against the metering roller 14 to remove all of the ink on the metering roller 14 except that in cells or interstices, when present. Ink from transfer roller 15 is passed onto a substantially smooth inking drum 20 where it is combined with water supplied from dampener 21. Dampening fluid can be supplied by any appropriate means, either to the ink roll 20 as shown or directly to the plate roll 25, as indicated by the phantom lines at 26. The scraping blade 16 (or other ink removal means) operating against the metering roll 13 is present to continuously remove substantially all of the excess ink film therefrom. All of the aforesaid elements function to supply a uniform film of ink to the printing plate 28 mounted on press driven plate cylinder 25. The plate on cylinder 25 in turn supplies ink in the form of an image, for example, to a paper web 30 being fed through the printing nip formed by the coacting blanket cylinder 31 and impression cylinder 32. All of the rollers in FIGS. 1 and 2 are configured substantially axially parallel.

Many other press configurations can be visualized by those skilled in the art and science of keyless lithographic printing, the primary features that are important for proper operation of this invention are discussed below.

The amount of ink reaching the printing plate may be controlled by the dimensions of depressions or of ink receiving cells formed in the surface of the ink metering roller in conjunction with a coextensive scraping or

doctor blade that continuously removes virtually all of the ink from the celled metering roller except that carried in the cells or recesses.

The ink metering roller is composed of a steel or aluminum or comparable core material of suitable strength, length and diameter that is suitably coated with a relatively thick wear-resistant ceramic material. While the roller surface need not be engraved in all instances, laser engraving can be used to form accurately dimensioned and positioned cells or recesses, which cells together with a scraping doctor blade serve to precisely meter a required volume of ink. To ensure accurate and continuous metering of ink by all regions of the roller surface of the wear-related useful lifetime 10 of the roller, the ceramic materials are infused with organic materials that react with their individual components to form a hydrophobic and oleophilic reaction product.

FIG. 2 is a cross-sectional view of one form of this invention in which the base roller used to produce metering roller 14 is engraved before application of the ceramic coating indicated by numeral 35.

The celled metering roller 14 illustrated in the drawings, may be, as previously mentioned, mechanically- 25 engraved and then coated or may be first coated and then laser-engraved to form patterned cells of depressions in the coated surface of the roller. The volume and frequency of the depressions are selected based on the volume of ink required to meet the printed optical density specifications and in accordance with known practices. Alternatively, the roller may have a nominally smooth face with the hard, oleophilic and hydrophobic surface properties added as herein described.

Roller 14 is employed typically together with a scraping or doctoring blade 16 to meter the input of ink into the press system. Roller 20 may instead be typically employed as the metering roller in a position closer to the printing plate and may function together with a scraping blade (not shown) that removes from the printing system virtually all of used return ink that exists at that location. Rollers 13 and 15 are then not needed. In either case the return film of ink, that is the unused portion of the input ink, is continuously scraped off and led to sump 10 for subsequent continuous recirculation 40 by pump 11 back to the celled metering roller 14. Many of these keyless lithography press operational elements are described in more detail in Fadner, et al U.S. Pat. No. 4,690,055.

I have found that the commonly available hard, wear-resistant ceramic and ceramic-like materials such as alumina, tungsten carbide or chromium oxide, all of which are available for manufacture of an inking roller, prefer to have a layer of water rather than a layer of oil-based ink on their surfaces when both liquids are present. Although various ceramic materials are known to function as the hard, wear-resistant uppermost surface of ink metering rollers either for a printing system such as letterpress involving a single oil-based printing fluid or for flexographic printing systems using a single water-based inking fluid, these same ceramic surfaces when used in lithographic printing will become debonded of an oil or resin-based ink whenever sufficient dampening water penetrates through the ink to the roller. This is more readily understood if one considers that hydrophilic or water-loving surfaces such as ceramic materials are, in the absence of water oleophilic or oil loving. When fresh, unused, water-free lithographic ink is applied to a ceramic, the ink initially

exhibits good adhesion to and wetting of the roller surface. Under these initial conditions, normal ink-metering performance is observed. However, during lithographic printing operations, as the water content in the ink increases, a condition is reached where a combination of roller nip pressure and increasing water content in the ink force water through the ink layer to the ceramic metering roller surface. By adhering preferentially to the rollers surface, the water debonds the ink from that surface, thereby disallowing subsequent pickup of ink from the ink input means.

I have found that water-interference problems associated with using state-of the-art ceramic-covered rollers to meter ink in keyless lithographic inking system can be avoided by fixedly applying to the ceramic roller's surface and infusing into the interstices of a microporous layer of ceramic material organic materials that react within their individual components to form a reaction product that possesses oleophilic and hydrophobic properties. Ceramic rollers thus treated function as metering rollers in lithographic printing systems without the aforementioned chemically-related ink metering failure.

In one form of this invention a steel or aluminum or other suitable roller may be mechanically engraved in patterns similar for instance to those shown in FIG. 2, then flame-spray ceramic coated to the maximum thickness that substantially retains the cell structure originally present in the core's surface, about 5 to 8 mils. In the case of a base roller manufactured of aluminum, the roller can be given a hard anodizing treatment to form the ceramic-like layer in situ. The deposition process normally requires repeated thin-application passes of the ceramic coating apparatus, and may be followed by infusion with a selected organic substance, as elsewhere described herein.

Alternatively, the roller core is similarly mechanically engraved, then one-pass flame spray coated with a thin film of ceramic powder to a coating thickness typically less than about 0.1 to 0.2 mil, then infused with the organic substances of this invention that subsequently react together to form an oleophilic and hydrophobic substantially solid material, then given another ceramic coating pass, then another infusion treatment and so on until the desired 5 to 8 mil thick ceramic coating is built-up by successive coating and infusion treatments.

The desired microporous layer can be obtained also by subjecting a steel or aluminum roller core to a multiple-pass flame-spray coating with the selected ceramic particles to build up a thick, from 3 to about 10 mil or more coating. This coating, such as indicated by numeral 40 in FIGS. 4 and 5, is then laser engraved to create cell patterns 41 for instance as depicted in FIGS. 4 and 5 after which the organic agents are infused into the ceramic surface.

The same sort of structure can be obtained where the organic agent is applied after each flame-spray coating pass in a series of about 6 to 20 or so sequences, to achieve the desired organic/ceramic coating thickness, then laser engraved to create the required ink carrying capacity.

Several types of oleophilic and hydrophobic material forming agents can be used, oleophilic and hydrophobic agents are here intended to mean those organic substances that can be infused into the microporous ceramic and as a more or less highly fluid or pair of liquids then reacted or cured, as by heating, ultraviolet radiation or the like, to form an immobilized solid that has

oleophilic and hydrophobic properties. These are generally dissolvable solids or liquids that can therefore be applied by mist, spray, dip or other well known application methods. One primary objective in providing the oleophilic and hydrophobic material is to render as much as possible of the microporous ceramic powder coating interstices and surfaces oil attracting and water repellent by penetration of the oleophilic and hydrophobic material as deep as possible into the porous ceramic coating. Highly mobile liquid systems are preferred. Simple spray-painting techniques are appropriate as are dip-coating with roller rotation. Dilute solutions of the reactive agent in solvents that allow seconds to minutes open time will help to provide penetration deep into the interstices of the ceramic coating.

In all cases, the oleophilic and hydrophobic material must be rendered essentially immobile and firmly physically adhered to ceramic surfaces or at least entrapped within the ceramic powder coating's voids. The objects of this invention are achieved through the infusion of organic materials that are chemically self-reactive to form hydrophobic and oleophilic materials but generally unreactive chemically to the ceramic coating material. Generally, these will be long chain hydrocarbons or substantially hydrocarbon polymeric materials having chemically reactive groups incorporated thereto. Materials which fulfill the requirements are all polymerization or coupling-reactive, substantially hydrocarbon, monomer, copolymer, prepolymer and the like that satisfy the finished roller contact angle criteria discussed hereafter. Particularly useful and practical are the reactive polystyrenes, polyisobutylenes, acrylonitrile-butadiene-styrenes, polybutadienes, nitrile rubbers and the like. Another suitable substance is the two part chemically reactive epoxy/amine system designated as 492×6215 produced and sold by the Pauert Chemical Co. Other useful oleophilic and hydrophobic materials of these classes will be apparent to those skilled in the chemical and polymeric sciences and based on the elements of this invention herein disclosed.

FIG. 6 of the drawings illustrates the manner in which the oleophilic and hydrophobic material is infused into the interstitial voids formed by the ceramic coating. In FIG. 6, numeral 50 indicates generally the composite wear resistant layer, while numeral 51 identifies the particles of ceramic material and numeral 52 the infused substance which is reacted by appropriate means to form the required oleophilic and hydrophobic reaction product. For a maximum useful life it is preferred that the entire interconnecting network of voids formed by the deposited ceramic layer be infused substantially completely throughout the volume of the ceramic cooling layer.

Notwithstanding certain general or specific material disclosure of organic agents which can be reacted together to form oleophilic and hydrophobic materials according to the practice of this invention, the important criterion for the resulting roller's use as a lithographic inking roller can be more-or less predicted by measuring the degree to which droplets of ink oil and of water will spontaneously spread out on the surface of the treated roller. The sessile drop technique as described in standard surface chemistry textbooks is suitable for measuring this quality. Generally, oleophilic and hydrophobic roller materials will have an ink oil (Flint Ink Co.) contact angle of nearly 0° and a distilled water contact angle of about 90° or higher and these

values serve to define an oleophilic and hydrophobic material.

I have found, for instance, that the following rules are constructive in but not restrictive for selecting materials according to this principle:

|              |                                                              |
|--------------|--------------------------------------------------------------|
| Best         | Water contact angle 90° or higher.                           |
| Maybe        | Ink Oil contact angle 10° or lower and spreading.            |
| Acceptable   | Water contact angle 80° or higher.                           |
| Probably Not | Ink Oil contact angle 10° or lower and spreading.            |
| Acceptable   | Water contact angle less than about 80°                      |
|              | Ink Oil contact angle greater than 10° and/or non-spreading. |

Materials that have this oleophilic and hydrophobic property as defined herein will in practice in a lithographic printing press configuration accept retain and maintain lithographic ink on their surface in preference to water or dampening solution when both ink and water are presented to or forced onto that surface. And it is this combined oleophilic and hydrophobic property that allows rollers used in lithographic press inking roller trains to assist in the transport of ink from an ink reservoir to the substrate being printed without loss of printed-ink density control due to debonding of the ink by water from one or more of the inking rollers.

I claim:

1. A wear-resistant ink metering roller possessing oleophilic and hydrophobic properties comprising:

- a. a base roller of preselected strength, diameter and length having an outer surface of substantially cylindrical shape;
- b. a substantially continuous microporous ceramic layer integral to the outer surface of said base roller, said microporous ceramic layer defining an interconnecting network of openings that permeate substantially the entire volume of said ceramic layer, said openings defining a void volume in said microporous ceramic layer; and
- c. an oleophilic and hydrophobic reaction product substantially filling said void volume and formed by a curing of a coupling-reactive material, said material being from the group consisting of reactive and polymerizable materials, substantially hydrocarbon monomer, copolymer and prepolymer materials that have a water contact angle of not less than 90° and an ink oil contact angle of not higher than 10° and spreading, said microporous ceramic layer containing said material being oleophilic and hydrophobic and said microporous ceramic layer having a plurality of thin coatings of ceramic material, each of said thin coatings of ceramic material having applied thereto said coupling reactive material.

2. An ink metering roller as defined in claim 1, wherein said oleophilic and hydrophobic reaction product is formed from the material selected from the group consisting of:

- a. polystyrenes;
- b. polyisobutylenes;
- c. acrylonitrile-butadiene-styrenes;
- d. polybutadienes; and
- e. nitrile rubbers.

3. An ink metering roller as defined in claim 1, wherein said oleophilic and hydrophobic reaction product is formed by the self-reaction of polystyrene as the material.

4. An ink metering roller as defined in claim 1, wherein said oleophilic and hydrophobic reaction prod-

uct is formed by the self-reaction of polyisobutylene as the material.

5. An ink metering roller as defined in claim 1, wherein said oleophilic and hydrophobic reaction product is formed by the self-reaction of acrylonitrile-butadiene-styrene as the material.

6. An ink metering roller as defined in claim 1, wherein said oleophilic and hydrophobic reaction product is formed by the self-reaction of polybutadiene as the material.

7. An ink metering roller as defined in claim 1, wherein said oleophilic and hydrophobic reaction product is formed by the self-reaction of nitrile rubber as the material.

8. In a process for producing a wear resistant ink metering roller possessing oleophilic and hydrophobic properties the steps comprising:

- a. providing a base roller having a substantially cylindrical surface microporous layer formed of a microporous ceramic material which defines an interconnecting network of openings that permeate substantially the entire volume of the microporous layer, said openings defining a void volume in said microporous ceramic material;
- b. infusing the void volume with a solute of a reactive organic material selected from the group consisting of reactive and polymerizable materials, substantially hydrocarbon monomer, copolymer and prepolymer materials that have a water contact angle of not less than 90° and ink oil contact angle of not higher than 10° and spreading; and
- c. subjecting said selected organic material to treatment causing it to react and form a substance in the interconnecting network that is oleophilic and hydrophobic thereby causing said microporous ceramic layer to be oleophilic and hydrophobic;
- d. the microporous ceramic layer being deposited on the base roller in incremental applications and each incremental layer being infused with the material prior to deposition of the next incremental part of the ceramic layer.

9. A keyless lithographic printing press system utilizing at least an oil based ink comprising:

- a. a base roller of preselected strength, diameter and length having an outer surface of substantially cylindrical shape;
  - b. a substantially continuous microporous ceramic layer integral on the outer surface of said base roller, said microporous ceramic layer defining an interconnecting network of openings that permeate substantially the entire volume of said ceramic layer, said openings defining a void volume in said microporous ceramic material; and
  - c. an oleophilic and hydrophobic reaction product formed by a curing of a coupling-reactive organic material infused into said void volume of said microporous ceramic layer and selected from the group consisting of:
- polystyrenes;  
polyisobutylenes;  
acrylonitrile-butadiene-styrenes  
polybutadienes;  
nitrile rubbers;
- d. scraper means mounted in reverse-angle relationship contact with said infused microporous ceramic coated base roller to remove at least excess ink therefrom; and

e. said microporous ceramic layer containing said reaction product being oleophilic and hydrophobic and said microporous ceramic layer having a plurality of thin coatings of ceramic material, each of said thin coatings of ceramic material having applied thereto said coupling reactive material.

10. In a process for producing a wear resistant ink metering roller possessing oleophilic and hydrophobic properties the steps comprising:

a. providing a base roller having a substantially cylindrical surface microporous layer formed of a microporous ceramic material which defines an interconnecting network of openings that permeate substantially the entire volume of the microporous 15 layer, said openings defining a void volume in said microporous ceramic material;

5  
b. infusing the void volume with a solute of a reactive organic material selected from the group consisting of reactive and polymerizable materials, substantially hydrocarbon monomer, copolymer and pre-polymer materials that have a water contact angle of not less than 90° and an ink oil contact angle of not higher than 10° and spreading; and  
c. subjecting said selected organic material to treatment causing it to react and form a substance in the interconnecting network that is oleophilic and hydrophobic;  
d. said microporous ceramic layer being deposited on the base roller in incremental applications and each incremental layer being infused with the reactive organic material prior to deposition of the next incremental part of the ceramic layer.

\* \* \* \* \*

20

25

30

35

40

45

50

55

60

65